

## [54] METHOD FOR DEVELOPING SILVER HALIDE EMULSIONS

[75] Inventor: Jozef Frans Willems, Wilrijk, Belgium

[73] Assignee: Afga-Gevaert, Mortsel, Belgium

[22] Filed: Oct. 7, 1970

[21] Appl. No.: 78,914

## [30] Foreign Application Priority Data

Oct. 27, 1969 Great Britain.....52,565/69

[52] U.S. Cl. ....96/29, 96/66, 96/66.3

[51] Int. Cl. ....G03c 5/54, G03c 5/30

[58] Field of Search ....96/66, 66 T, 55, 29

## [56] References Cited

## UNITED STATES PATENTS

|           |         |                  |       |
|-----------|---------|------------------|-------|
| 3,489,566 | 1/1970  | Anselm .....     | 96/22 |
| 2,857,274 | 10/1958 | Land .....       | 96/29 |
| 2,857,275 | 10/1958 | Land .....       | 96/29 |
| 3,113,866 | 12/1963 | Land .....       | 96/29 |
| 3,406,064 | 10/1968 | Land .....       | 96/29 |
| 3,576,631 | 4/1971  | Archambault..... | 96/66 |
| 3,265,499 | 8/1966  | Willems.....     | 96/66 |
| 3,265,502 | 8/1966  | Willems.....     | 96/66 |
| 3,549,364 | 12/1970 | Morse .....      | 96/66 |

Primary Examiner—J. Travis Brown

Assistant Examiner—M. F. Kelley

Attorney—Brufsky, Staas, Breiner and Halsey

## [57] ABSTRACT

A photographic developing method is described which comprises developing an exposed silver halide emulsion layer of a photographic material with an aqueous alkaline composition in the presence of a hydroxylamine developing agent and a p-phenylene diamine or p-aminophenol derivative corresponding to one of the formulas



wherein:

R<sub>1</sub> stands for an alkyl group,  
 R<sub>2</sub> stands for alkyl or for ethylene, substituted ethylene, propylene or substituted propylene attached to the adjacent ortho-carbon atom of the benzene ring,

R<sub>3</sub> stands for alkyl, and

R<sub>4</sub> stands for an alkyl group,  
 at most one of R<sub>1</sub> and R<sub>4</sub> being substituted alkyl;



wherein:

each of R<sub>5</sub> and R<sub>6</sub> stands for an alkyl group, and  
 X<sub>1</sub> stands for an electron-donating group; and



wherein:

each of X<sub>2</sub> and X<sub>3</sub> stands for hydrogen, halogen or an electron-donating group,

Y stands for OH or NH<sub>2</sub>, and

R<sub>7</sub> stands for ethylene, substituted ethylene, propylene or substituted propylene attached to the adjacent ortho-carbon atom of the benzene ring, and

R<sub>8</sub> stands for hydrogen, an alkyl group or has the same significance as R<sub>7</sub>, or

R<sub>7</sub> together with R<sub>8</sub> and the N-atom to which they are attached from a pyrrolidine ring.

The p-phenylene diamine or p-aminophenol derivative has a super-additive developing effect with the hydroxyl amine developing agent.

10 Claims, No Drawings

**METHOD FOR DEVELOPING SILVER HALIDE  
EMULSIONS**

This invention relates to the development of photographic materials containing exposed silver halide, to new developing combinations and to photographic materials and solutions containing such combinations.

It is known that certain chemical compounds, which used alone are poor developers for photographic silver halide emulsions, become much more effective when used in conjunction with other developers, the effect being known as superadditivity. Thus, for example it is known that p-phenylene diamine derivatives and p-aminophenol derivatives show the phenomenon of superadditivity when used in conjunction with developing agents the ionized forms of which in alkaline medium carry two or more negative charges such as hydroquinone, hydroquinone sulphonate, ascorbic acid, etc.

It has now been found that these p-phenylene diamine and p-aminophenol derivatives also exhibit a superadditive character when used in conjunction with the at most singly ionized developer anions of hydroxylamine and derivatives thereof.

The use of hydroxylamine and derivatives thereof, of which the oxidation products have the favorable property of leaving no residual stain in the silver image obtained has been disclosed amongst others in U.S. Pat. No. 2,857,276 of Edwin H. Land and Helen J. Tracy issued Oct. 21, 1958. Hydroxylamine itself and the mono-alkyl derivatives are less suitable because they can give rise to fog but the N,N-dialkylhydroxylamines such as N,N-diethylhydroxylamine and the heterocyclic N-hydroxylamines such as N-hydroxymorpholine, N-hydroxypiperidine and N-hydroxypyrrrolidine disclosed in the above United States Patent Specification are particularly suitable. Other hydroxylamine derivatives that have been proposed for use as silver halide developing agents and of which the development activity is higher than that of the N,N-di-alkyl hydroxylamines include for example aminoalkyl hydroxylamines, more especially N,N-diethylhydroxylamines having in at least one of the N-alkyl groups an intralinear amino nitrogen atom, either cyclic or acyclic, examples of which can be found in U.S. Pat. No. 3,287,125 of Milton Green, Adnan A. Sayigh and Henri Ulrich issued Nov. 22, 1966, alkoxyhydroxylamines, more especially N,N-diethylhydroxylamines of which at least one of the n-alkyl groups is substituted by alkoxy or alkoxyalkoxy, examples of which can be found in U.S. Pat. No. 3,293,034 of Milton Green, Adnan A. Sayigh and Henri Ulrich issued Dec. 20, 1966 and sulphone hydroxylamines, more especially N,N-di-alkylhydroxylamines having in at least one of the N-alkyl groups an intralinear sulphonyl ( $-\text{SO}_2-$ ) group, examples of which can be found in U.S. Pat. No. 3,287,124 of Milton Green, Adnan A. Sayigh and Henri Ulrich issued Nov. 22, 1966. Further N,N-diethylhydroxylamines having in at least one of the N-alkyl groups a quaternary ammonium group either cyclic or acyclic which excel by their high development activity have been proposed for use as silver halide developing agents in the copending application filed for "Novel Photographic Developers" (=U.K. Pat. Application No. 52,564/69 filed Oct. 27, 1969 by Gevaert-Agfa N.V.).

The p-phenylene diamine and p-aminophenol derivatives having a superadditive development effect with

hydroxylamine developing agents can be represented by the following general formulae:

I.



wherein:

R stands for alkyl including substituted alkyl, e.g., substituted by hydroxy, carboxy, sulpho, sulphate, acylamino and sulphonamido such as methyl, ethyl, propyl, butyl, pentyl, hexyl, 2-hydroxyethyl, 3-hydroxypropyl, 4-hydroxybutyl, 4-carboxybutyl, 5-carboxyhexyl, 4-sulphobutyl, 5-sulphatopentyl, 2-acylaminethyl, 2-methylsulphonylaminethyl, etc.

R<sub>2</sub> stands for alkyl or for ethylene, substituted ethylene, propylene, or substituted propylene attached to the adjacent ortho-carbon atom of the benzene ring,

R<sub>3</sub> stands for alkyl, and

R<sub>4</sub> stands for alkyl including substituted alkyl for instance as exemplified for R<sub>1</sub> at most one of R<sub>1</sub> and R<sub>4</sub> being substituted alkyl,

II.



wherein:

each of R<sub>5</sub> and R<sub>6</sub> stands for alkyl including substituted alkyl e.g., alkyl substituted as above, and

X<sub>1</sub> stands for an electron-donating group such as alkyl, alkoxy, amino, monoalkylamino, dialkylamino, acylamino and sulphonamido,

III.



wherein:

each of X<sub>2</sub> and X<sub>3</sub> stands for hydrogen, halogen such as chlorine or an electron donating group, e.g., as exemplified for X<sub>1</sub>,

Y stands for OH or NH<sub>2</sub>, and

R<sub>7</sub> stands for ethylene, substituted ethylene, propylene or substituted propylene attached to the adjacent ortho-carbon atom of the benzene ring, and

R<sub>8</sub> stands for hydrogen, alkyl including substituted alkyl for instance substituted as exemplified above for R<sub>1</sub>, or has the same significance as R<sub>7</sub> above, or

R<sub>7</sub> together with R<sub>8</sub> and the N-atom to which they are attached form a pyrrolidine ring.

The following are representative examples of p-phenylene diamine and p-aminophenol derivatives

suitable for use as superadditive developing agents in conjunction with hydroxylamine

a. compounds corresponding to general formula I

1. 6-diethylamino-1,2,3,4-tetrahydroquinoline dichlorohydrate
2. 1-ethyl-6-diethylamino-1,2,3,4-tetrahydroquinoline dichlorohydrate
3. 1-(4-sulphobutyl)-6-diethylamino-1,2,3,4-tetrahydroquinoline
4. 1-(2-hydroxyethyl)-6-dimethylamino-1,2,3,4-tetrahydroquinoline dichlorohydrate
5. 1-ethyl-6-(N-ethyl-N-3-sulphopropylamino)-1,2,3,4-tetrahydroquinoline dichlorohydrate
6. 11(3-sulphopropyl)-6-(N-ethyl-N-methylamino)-1,2,3,4-tetrahydroquinoline dichlorohydrate
7. 1-(2methylsulphonylaminooethyl)-6-diethylamino-1,2,3,4-tetrahydroquinoline dichlorohydrate
8. 1-(3-carboxypropyl)-6-dimethylamino-1,2,3,4-tetrahydroquinoline dichlorohydrate
9. N,N-diethyl-N',N'-dimethyl-p-phenylene diamine dihydrochloride
10. N,N,N', N'-tetramethyl-p-phenylene diamine dihydrochloride
11. N,N,N', N'-tetraethyl-phenylene diamine dihydrochloride
12. N,N-diethyl-N'-2-hydroxyethyl-N'-ethyl-p-phenylenediamine disulphate
13. N,N-diethyl-N'-4-sulphobutyl-N'-ethyl-p-phenylene diamine

b. compounds corresponding to general formula II

14. 2-amino-4-diethylamino-aniline sulphate
15. 2-methylamino-4-diethylamino-aniline sulphate
16. 2-methylsulphonamido-4-diethylamino-aniline sulphate
17. 2-ethoxy-4-diethylamino-aniline hemisulphate
18. 1-(4-hydroxyphenyl)-pyrrolidine
19. 1-(3-chloro-4-hydroxyphenyl)-pyrrolidine
20. 1-(3-methyl-4-hydroxyphenyl)-pyrrolidine
21. 1-(3,5-dimethyl-4-hydroxyphenyl)-pyrrolidine
22. 1-(3-amino-4-hydroxyphenyl)-pyrrolidine
23. 1-(3-methoxy-4-hydroxyphenyl)-pyrrolidine
24. 1-(3-methylsulphonamido-4-hydroxyphenyl)-pyrrolidine
25. 1-(3-acetylamino-4-hydroxyphenyl)-pyrrolidine
26. 6-amino-1,2,3,4-tetrahydroquinoline
27. 6-hydroxy-1,2,3,4-tetrahydroquinoline
28. 1-ethyl-6-hydroxy-1,2,3,4-tetrahydroquinoline chlorohydrate
29. 1-(4-sulphobutyl)-6-hydroxy-1,2,3,4-tetrahydroquinoline
30. 9-amino-julolidine sulphate

31. 1-methyl-6-amino-1,2,3,4-tetrahydroquinoline oxalate

32. 1-(2-methylsulphonylaminooethyl)-6-hydroxy-1,2,3,4-tetrahydroquinoline
33. 1-(2-hydroxyethyl)-6-hydroxy-1,2,3,4-tetrahydroquinoline
34. 1-(4-sulphobutyl)-6-amino-1,2,3,4-tetrahydroquinoline
35. 9-hydroxy-julolidine.

The p-phenylene diamine and p-aminophenol compounds of use according to the present invention can be prepared as known in the art, e.g. as described in U.S. Pat. No. 3,265,499 of Jozef Frans Willems,

George Frans Van Veen and Louis Maria De Haes issued Aug. 9, 1966 and U.S. Pat. No. 3,265,502 of Jozef Frans Willems and George Frans Van Veen issued July 8, 1966, in United Kingdom Pat. specifications, 5 No. 928,671 filed Feb. 19, 1960 by Ilford Ltd. and No. 858,432 filed Mar. 5, 1958 by Imperial Chemical Industry and in Belgian Pat. specification No. 715,500 filed May 22, 1968 by Gevaert-Agfa N.V.

In accordance with the present invention there is provided a process of making photographic records which comprises treating a photographic material having layers containing developable silver salts with an aqueous alkaline solution in the presence of a hydroxylamine developing agent and a p-phenylene diamine or p-aminophenol compound as described above. The invention also includes developer compositions comprising in addition to a hydroxylamine developing agent, a p-phenylene diamine or p-aminophenol compound as described. By hydroxylamine developing agent it is intended to embrace hydroxylamine itself as well as derivatives thereof as described above. The p-phenylene diamine and p-aminophenol derivative of use according to the present invention may be added to the developing bath or to the emulsion or to both simultaneously, the processing bath being preferred, however.

Developer compositions that comprise the superadditive developing agents according to the present invention may comprise in addition thereto any of the common ingredients employed in developing compositions, e.g., alkalies such as sodium hydroxide, potassium hydroxide, sodium carbonate, trisodium phosphate etc., silver halide solvents such as sodium thiosulphate, sodium thiocyanate and cyclic imides such as barbiturates or uracils, preservatives such as sulphites, bisulphites, metabisulphites and acids such as boric acid and citric acid. Further the developer composition may comprise potassium bromide and water-softening agents such as polyphosphates and derivatives of ethylene diamine tetraacetic acid, antifoggants such as benzotriazole, 5-nitrobenzotriazole and 6-nitrobenzimidazole and wetting agents as well as other compounds known in the photographic development technique such as development restrainers and development accelerators.

The ratio of hydroxylamine developing agent to p-phenylene diamine or p-aminophenol compound used in the present invention can be chosen in such a way that the combination is suited for the development of all kinds of materials including materials having silver chloride emulsion layers of low sensitivity as well as materials having highly sensitive silver bromo-iodide emulsion layers. This ratio may vary within wide limits and also depends on the particular hydroxylamine developing agent used. In most cases the ratio is chosen in such a way that the amount of the hydroxylamine developing agent strongly outweighs the p-phenylene diamine or p-aminophenol compound.

A strong superadditive effect is obtained by using an amount of 0.05 to 10 millimole preferably from 0.3 to 6 millimole of p-phenylene diamine or p-aminophenol derivative to an amount of 10 to 100 millimole of hydroxylamine developing agent, per liter of developing composition. Of course larger amounts of said p-phenylene diamine or p-aminophenol compounds can

be used, although the superadditive effect obtained with higher concentrations is not more considerable.

The novel combination of developing agents of the invention may be used in conventional or wet development of silver halide emulsions, in diffusion transfer processes, both dye and silver, in such photographic processes known as stabilization processing wherein it is desired to eliminate or minimize the need for washing or stabilizing operations in liquid baths subsequent to the formation of the silver print, etc.

In diffusion transfer processes, as is well known in the art, an exposed silver halide emulsion is treated with a liquid processing composition while in superposed relationship with an image-receiving material. By this treatment the exposed silver halide is developed to silver and the unexposed silver halide is converted into a complex silver salt which is transferred to the image-receiving material and there reduced to silver to form a positive print. The processing composition normally includes a silver halide solvent, such as sodium thiosulphate, sodium thiocyanate and cyclic imides such as barbiturates or uracils, which forms with silver halide a soluble complex as is well known in the art of forming silver images by transfer, and may also include a film-forming material such as sodium carboxymethylcellulose and hydroxyethylcellulose, starch or gum for increasing the viscosity of the composition as, for instance, in the case of in-camera silver complex diffusion transfer processing.

In stabilization processing the time-consuming fixing and washing operations are eliminated in order to produce the photographic record in the least possible time by converting after development, with the aid of stabilizing agents such as ammonium thiocyanate, the unexposed and undeveloped silver halide of the photographic emulsion into colorless light-insensitive compounds that need not be removed by washing.

The developing agents of use according to the invention may be employed in solution or they may be initially incorporated in a layer of the photosensitive material, e.g., a silver halide emulsion layer or an other colloid layer in water-permeable relationship therewith. In silver complex diffusion transfer processes they may also be incorporated in a layer of the image-receiving material which, during processing, is in superposed relationship with the photosensitive silver halide material.

The following examples illustrate the present invention.

#### Example 1

Strips of a photographic material comprising a light-sensitive silver halide emulsion layer coated on a cellulose triacetate support are exposed through a grey filter with a light-quantity (E) which corresponds to the shoulder part of the density/log E curve.

Each of the exposed strips is developed at 20°C in a separate developing bath. One of them is developed in a bath A containing as developing agent only hydroxylamine hydrochloride and having the following composition:

|                             |           |
|-----------------------------|-----------|
| sodium sulphite             | 100 g     |
| sodium hydroxide            | 10 g      |
| 5-nitro-benzotriazole       | 80 mg     |
| potassium bromide           | 1 g       |
| hydroxylamine hydrochloride | 0.06 mole |

water to make 1 liter

The other strips are developed in baths having the same composition as bath A but containing moreover one of the compounds listed in the table below in the amount given.

The densities obtained are listed in the following table.

| 10                                         | Developing bath | Densities obtained after a development time of |       |      |      |
|--------------------------------------------|-----------------|------------------------------------------------|-------|------|------|
|                                            |                 | 0sec                                           | 20sec | 1min | 3min |
| Bath A                                     | 0.04            | 0.05                                           | 0.34  | 0.95 | 1.43 |
| Bath A + 105 mg (0.31 mmole) of compound 3 | 0.04            | 0.07                                           | 0.79  | 1.97 | 2.68 |
| Bath A + 66 mg (0.31 mmole) of compound 28 | 0.04            | 0.12                                           | 0.86  | 2.17 | >3   |

#### Example 2

This example is analogous to example 1 with the only difference that now a developing bath B is used which only differs from bath A in that the hydroxylamine hydrochloride has been replaced by 0.06 mole of N-methylhydroxylamine hydrochloride.

The following results are attained.

| 30                                         | Developing bath | Densities obtained after a development time of |       |      |      |
|--------------------------------------------|-----------------|------------------------------------------------|-------|------|------|
|                                            |                 | 0sec                                           | 20sec | 1min | 3min |
| Bath B                                     | 0.05            | 0.05                                           | 0.07  | 0.60 | 1.09 |
| Bath B + 105 mg (0.31 mmole) of compound 3 | 0.04            | 0.04                                           | 0.19  | 1.83 | 2.61 |
| Bath B + 66 mg (0.31 mmole) of compound 28 | 0.04            | 0.04                                           | 0.18  | 1.66 | 2.72 |

#### Example 3

This example is analogous to example 1 with the only difference that now a developing bath C is used which only differs from bath A in that the hydroxylamine hydrochloride has been replaced by 0.06 mole of N,N-diethylhydroxylamine oxalate.

The following results are attained.

| 50                                         | Developing bath | Densities obtained after a development time of |       |      |      |
|--------------------------------------------|-----------------|------------------------------------------------|-------|------|------|
|                                            |                 | 0sec                                           | 20sec | 1min | 3min |
| Bath C                                     | 0.04            | 0.04                                           | 0.04  | 0.07 | 0.37 |
| Bath C + 105 mg (0.31 mmole) of compound 3 | 0.04            | 0.04                                           | 0.11  | 1.55 | 2.37 |
| Bath C + 55 mg (0.31 mmole) of compound 14 | 0.04            | 0.04                                           |       | 0.49 | 1.27 |
| 0.09                                       |                 |                                                |       |      |      |
| Bath C + 66 mg (0.31 mmole) of compound 28 | 0.04            | 0.04                                           | 0.07  | 0.81 | 2.03 |
| Bath C + 88 mg (0.31 mmole) of compound 34 | 0.04            | 0.04                                           | 0.05  | 0.32 | 1.07 |

#### Example 4

This example is analogous to example 1 with the only difference that now a developing bath D is used which only differs from bath A in that the hydroxylamine hydrochloride has been replaced by 0.06 mole of N-methyl-N-(2-hydroxy-3-diethylaminopropyl) hydroxylamine.

The following results are attained.

| Developing bath                            | Densities obtained after a development time of |       |      |      |      |
|--------------------------------------------|------------------------------------------------|-------|------|------|------|
|                                            | 0sec                                           | 20sec | 1min | 3min | 5min |
| Bath D                                     | 0.04                                           | 0.04  | 0.04 | 0.11 | 0.56 |
| Bath D + 105 mg (0.31 mmole) of compound 3 | 0.04                                           | 0.04  | 0.17 | 1.33 | 2.15 |
| Bath D + 66 mg (0.31 mmole) of compound 28 | 0.04                                           | 0.04  | 0.12 | 1.01 | 1.97 |

## Example 5

This example is analogous to example 1 with the only difference that now a developing bath E is used which only differs from bath A in that the hydroxylamine hydrochloride has been replaced by 0.06 mole of the hydroxylamine derivative corresponding to the formula:



according to the co-pending application filed on even date herewith for "Novel Photographic Developers."

The following results are attained.

| Developing bath                            | Densities obtained after a development time of |       |      |      |      |
|--------------------------------------------|------------------------------------------------|-------|------|------|------|
|                                            | 0sec                                           | 20sec | 1min | 3min | 5min |
| Bath E                                     | 0.04                                           | 0.04  | 0.20 | 1.29 | 2.08 |
| Bath E + 105 mg (0.31 mmole) of compound 3 | 0.04                                           | 0.06  | 0.95 | 2.50 | >3   |
| Bath E + 66 mg (0.31 mmole) of compound 28 | 0.04                                           | 0.09  | 1.00 | 2.37 | >3   |

## Example 6

This example is analogous to example 1 with the only difference that now a developing bath F is used which only differs from bath A in that the hydroxylamine hydrochloride has been replaced by 0.06 mole of the hydroxylamine derivative with formula:



according to the co-pending application filed on even date herewith for "Novel Photographic Developers."

The following results are attained.

| Developing bath                            | Densities obtained after a development time of |       |      |      |      |
|--------------------------------------------|------------------------------------------------|-------|------|------|------|
|                                            | 0sec                                           | 20sec | 1min | 3min | 5min |
| Bath F                                     | 0.04                                           | 0.50  | 1.13 | 2.19 | >3   |
| Bath F + 105 mg (0.31 mmole) of compound 3 | 0.04                                           | 0.71  | 1.35 | 2.91 | >3   |
| Bath F + 66 mg (0.31 mmole) of compound 28 | 0.04                                           | 0.73  | 1.35 | 2.60 | >3   |

## Example 7

A photosensitive element was prepared comprising on a paper support a propylene, bromoiodide emulsion layer containing per kg an amount of silver halide corresponding to 60 g of silver nitrate.

After exposure, the photosensitive element and an image-receiving element, which comprises a silver receptive layer containing development nuclei dispersed in a matrix of colloidal silica coated on a water-impervious support according to the practice described in U.S. Pat. No. 2,823,122 of Edwin H. Land issued Feb. 11, 1958, were advanced in superposed relationship between a pair of pressure applying rollers to spread between them in a thin layer the following processing composition:

|                                  |           |
|----------------------------------|-----------|
| water                            | 100 ml    |
| sodium carboxymethylcellulose    | 5 g       |
| sodium hydroxide                 | 15 g      |
| uracil                           | 11.25 g   |
| 15 30 % ammonium hydroxide       | 3.5 ml    |
| N,N-diethylhydroxylamine oxalate | 0.06 mole |
| 1-phenyl-2-tetrazoline-5-thione  | 0.2 g     |
| compound 3                       | 105 mg    |

After a contact period of 36 seconds the emulsion 20 together with the layer of processing liquid was stripped from the image-receiving element to uncover the positive print.

When using a same developing composition but comprising no compound 3 the density of the positive print obtained was markedly lower. Moreover, in the presence of compound 3 better quality transfer images are obtained at lower illumination levels than is the case when using N,N-diethylhydroxylamine alone.

We claim:

- 30 1. Photographic developing method which comprises the black and white development of an exposed silver halide emulsion layer of a photographic material with an aqueous alkaline composition comprising a hydroxylamine developing agent and a p-phenylene diamine or p-aminophenol derivative having one of the formulas I, II and III:



wherein:

R<sub>1</sub> stands for an alkyl group,

R<sub>2</sub> stands for alkyl or an ethylene group, or a propylene group attached to the adjacent ortho-carbon atom of the benzene ring,

R<sub>3</sub> stands for alkyl, and

R<sub>4</sub> stands for an alkyl group, at most one of R<sub>1</sub> and R<sub>4</sub> being substituted alkyl,

55 II.



wherein:

- 65 each of R<sub>5</sub> and R<sub>6</sub> stands for an alkyl group, and X<sub>1</sub> stands for an electron-donating group selected from the group consisting of alkyl, alkoxy, amino, monoalkylamine, dialkylamine, acylamino, and sulphonamido,



wherein:

each of  $X_2$  and  $X_3$  stands for hydrogen, halogen or an electron-donating group selected from the group consisting of alkyl, alkoxy, amino, monoalkylamine, dialkylamino, acylamino, and sulphonamido,

$Y$  stands for  $\text{OH}$  or  $\text{NH}_2$ , and

$R_7$  stands for an ethylene or propylene group attached to the adjacent ortho-carbon atom of the benzene ring, and

$R_8$  stands for hydrogen, an alkyl group or has the same significance as  $R_7$ , or

$R_7$ , together with  $R_8$  and the N-atom to which they are attached from a pyrrolidine ring.

2. Photographic developing method according to claim 1, wherein said method is used for making images according to the silver complex diffusion transfer process.

3. Photographic developing composition for the black and white development of an exposed silver halide emulsion layer of a photographic material comprising in aqueous alkaline solution an hydroxylamine developing agent and a p-phenylene diamine or p-aminophenol derivative having one of the formulas I, II and III:



wherein:

$R_1$  stands for an alkyl group,

$R_2$  stands for alkyl or an ethylene group, or a propylene group attached to the adjacent ortho-carbon atom of the benzene ring,

$R_3$  stands for alkyl, and

$R_4$  stands for an alkyl group, at most one of  $R_1$  and  $R_4$  being substituted alkyl,



wherein:

each of  $R_5$  and  $R_6$  stands for an alkyl group, and

$X_1$  stands for an electron-donating group selected from the group consisting of alkyl, alkoxy, amino, monoalkylamine, dialkylamino, acylamino, and sulphonamido,

each of  $X_2$  and  $X_3$  stands for hydrogen, halogen or an electron-donating group selected from the group consisting of alkyl, alkoxy, amino, monoalkylamine, dialkylamino, acylamino, and sulphonamido,

$Y$  stands for  $\text{OH}$  or  $\text{NH}_2$ , and

$R_7$  stands for an ethylene or propylene group attached to the adjacent ortho-carbon atom of the benzene ring, and

$R_8$  stands for hydrogen, an alkyl group or has the same significance as  $R_7$ , or

$R_7$ , together with  $R_8$  and the N-atom to which they are attached from a pyrrolidine ring said p-phenylene diamine or p-aminophenol derivative being present in an amount of from 0.05 to 10 millimoles per 10 to 100 millimoles of hydroxyl amine developing agent per liter of developing composition.

4. Photographic developing method according to claim 1, wherein one of said hydroxylamine developing

30 agent and said p-phenylene diamine or p-aminophenol derivative is initially present in said photographic material and transferred to said aqueous alkaline composition therefrom.

5. The photographic developing method of claim 1 35 wherein said p-phenylene diamine or p-aminophenol derivative has the formula:



wherein:

$R_1$  stands for an alkyl group,

$R_2$  stands for alkyl or an ethylene group, or a propylene group attached to the adjacent ortho-carbon atom of the benzene ring,

$R_3$  stands for alkyl, and

$R_4$  stands for an alkyl group, at most one of  $R_1$  and  $R_4$  being substituted alkyl.

55 6. The photographic developing method of claim 1 wherein said p-phenylene diamine or p-aminophenol derivative has the formula:



wherein:

each of  $R_5$  and  $R_6$  stands for an alkyl group, and

$X_1$  stands for an electron-donating group selected

11

from the group consisting of alkyl, alkoxy, amino, monoalkylamine, dialkylamino, acylamino, and sulphonamido.

7. The photographic developing method of claim 1 wherein said p-phenylene diamine or p-aminophenol derivative has the formula:

III.



5

at most one of R<sub>1</sub> and R<sub>4</sub> being substituted alkyl.

9. Photographic developing composition of claim 3 wherein said p-phenylene diamine or p-aminophenol derivative has the formula:

II.



10

wherein:

each of X<sub>2</sub> and X<sub>3</sub> stands for hydrogen, halogen or an electron-donating group selected from the group consisting of alkyl, alkoxy, amino, monoalkylamine, dialkylamino, acylamino, and sulphonamido,

Y stands for OH or NH<sub>2</sub>, and

R<sub>7</sub> stands for an ethylene or propylene group attached to the adjacent ortho-carbon atom of the benzene ring, and

R<sub>8</sub> stands for hydrogen, an alkyl group or has the same significance as R<sub>7</sub>, or

R<sub>7</sub> together with R<sub>8</sub> and the N-atom to which they are attached from a pyrrolidine ring.

8. Photographic developing composition of claim 3 wherein said p-phenylene diamine or p-aminophenol derivative has the formula:

I.



20

15 wherein:

each of R<sub>5</sub> and R<sub>6</sub> stands for an alkyl group, and X<sub>1</sub> stands for an electron-donating group selected from the group consisting of alkyl, alkoxy, amino, monoalkylamine, dialkylamino, acylamino, and sulphonamido.

10. Photographic developing composition of claim 3 wherein said p-phenylene diamine or p-aminophenol derivative has the formula:

III.



25

wherein:

R<sub>1</sub> stands for an alkyl group,

R<sub>2</sub> stands for alkyl or an ethylene group, or a propylene group attached to the adjacent ortho-carbon atom of the benzene ring,

R<sub>3</sub> stands for alkyl, and

R<sub>4</sub> stands for an alkyl group,

35 wherein:

each of X<sub>2</sub> and X<sub>3</sub> stands for hydrogen, halogen or an electron-donating group selected from the group consisting of alkyl, alkoxy, amino, monoalkylamine, dialkylamino, acylamino, and sulphonamido,

40

Y stands for OH or NH<sub>2</sub>, and

R<sub>7</sub> stands for an ethylene or propylene group attached to the adjacent ortho-carbon atom of the benzene ring, and

R<sub>8</sub> stands for hydrogen, an alkyl group or has the same significance as R<sub>7</sub>, or

R<sub>7</sub> together with R<sub>8</sub> and the N-atom to which they are attached from a pyrrolidine ring.

\* \* \* \* \*

50

55

60

65